

## UNITED STATES PATENT OFFICE

2,434,048

MANUFACTURE OF ALLOYS CONTAINING  
MOLYBDENUM

George Leslie Miller, Hornchurch, England, assignor to Murex Limited, a corporation of Great Britain

No Drawing. Application February 21, 1945,  
Serial No. 579,155. In Great Britain March 8,  
1943

10 Claims. (Cl. 75—3)

**1** This invention relates to the manufacture of ferrous alloys containing molybdenum and more particularly to the production of a compact form of a molybdenum oxide suitable for use therein.

Many substances added to molten metals for the purposes of introducing an alloying ingredient are only commonly available in finely divided or powder form. In the addition of such substances the powder may suffer serious loss from the surface of the melt before it is incorporated, and it is well known to be desirable to introduce the substance into the body of the melt and well below the surface thereof. Thus for example the substance may be added in the form of a briquette or enclosed in a container constructed of some material which may itself be introduced into the melt without detriment thereto, e. g., an iron container in the case of a ferrous melt.

In the case of molybdenum alloys it has been proposed to introduce the molybdenum in the form of roasted molybdenite concentrates briquetted with the aid of a relatively small proportion of a carbonaceous binder which proportion may if desired be so adjusted as to provide an amount of carbon stoichiometrically equivalent to the oxygen content of the roasted molybdenite concentrates.

The principal object of the present invention is to provide a simple and economical process for the manufacture of compact forms of a molybdenum oxide having a high degree of hardness and strength. A further object of the invention is to provide novel compacts of a molybdenum oxide free from carbonaceous ingredient and having a high degree of hardness and strength. Yet a further object of the invention is to provide an improved process for the manufacture of ferrous alloys containing molybdenum. Other objects will appear hereinafter.

I have now found that it is possible to form briquettes of molybdenum trioxide ( $MoO_3$ ) or other molybdenum oxide merely with the aid of an aqueous solution of ammonia, or ammonium molybdate, and that the briquettes so produced have a surprising degree of hardness and represent a particularly convenient form in which to add the molybdenum oxide to a metallic melt since the ammonia is driven off at a temperature much below that of the melt and no non-volatile elements other than molybdenum and oxygen are incorporated into the bath. Ferrous melts to which molybdenum trioxide is to be added usually have a sufficient content of carbon and/or other reducing agents, such as manganese or silicon, to

reduce the oxide and I have found that it is simpler to adjust the composition of the melt by adding molybdenum trioxide alone than by endeavouring to balance the oxygen content with a proportion of carbon additional to that already present in the bath. Moreover, I have found that a more uniform and speedy reduction of the molybdenum trioxide takes place by means of the reducing agents of the ferrous melt with which the oxide comes into immediate and intimate contact than by means of an added carbonaceous ingredient. I have also found that the degree of hardness of the briquettes necessary to withstand rough handling can be achieved at relatively low pressures with consequent important economies in dies or moulds and other installation and maintenance costs.

According to the present invention I produce firm, coherent compact masses of a molybdenum oxide by pressing the oxide in powder form in the presence of an aqueous solution of an ammonium molybdate and drying the pressed product. The ammonium molybdate may be introduced, i. e., incorporated, into admixture with the molybdenum oxide either by addition in the form of an aqueous solution or by reaction in situ between the molybdenum oxide and ammonia added in the form of an aqueous solution thereof. Preferably I employ a proportion of ammonia or ammonium molybdate (calculated as  $NH_3$ ) lying between .05 per cent. and 2 per cent. by weight of the weight of the molybdenum oxide. In general the hardness and strength of the product increases with the amount of ammonia added, although it will be understood that the use of an undue proportion of ammonia is uneconomic.

In that form of the invention which comprises adding aqueous ammonia to the molybdenum oxide, I prefer to employ aqueous ammonia having a concentration lying between 5 per cent. and 33 per cent. by weight. The concentration of the ammonia should be so chosen as to afford a suitable proportion of water in the mix for good pressing characteristics; that is to say, independently of the proportion of ammonia ( $NH_3$ ) added, the proportion of water should not be so small that the mixture is too dry to press, and should not be so large that the mixture is too wet to press.

Pressures lying between 2 and 20 tons per square inch are suitable, more particularly pressures lying between 2 and 5 tons per square inch. For these pressures the proportion of water may suitably lie between .7 per cent. and 5 per cent.

by weight of the molybdenum oxide. In general an increase in pressure permits of the employment of a smaller proportion of water. In practice I find it convenient to add about  $\frac{1}{2}$  to 1 per cent. by weight of aqueous ammonia of 0.880 specific gravity diluted with its own volume of water. It is convenient to distribute the aqueous medium throughout the oxide by agitating the latter in a mixing device while the solution is sprayed over the charge. The mixed materials may then be formed into briquettes or other masses of convenient size and shape.

According to a further feature of the invention molybdenum is introduced as an alloying ingredient into molten metal baths containing carbon and/or other reducing agent such as manganese or silicon in solution by adding thereto an oxide of molybdenum in the form of a firm coherent pressed mass obtained in accordance with the process described and claimed herein.

The invention is illustrated but not limited by the following example.

A charge of 100 lbs. of molybdenum trioxide is introduced into a mixer and an aqueous solution of ammonia is sprayed over the charge while it is being mixed. The ammonia solution consists of 0.66 lb. of aqueous ammonia of 0.880 specific gravity diluted with 0.75 lb. of water. The mixing operation is continued until the ammonia solution is uniformly distributed throughout the charge. The moist charge is then briquetted at a pressure of 3 tons per square inch and the briquettes dried in a drying oven for a period of 3 to 8 hours at a temperature of  $120^{\circ}$  C. The briquettes so produced have a density of 200 lbs. per cubic foot as compared with a bulk density of the molybdenum trioxide powder of 100 lbs. per cubic foot.

I claim:

1. A process for the production of firm coherent masses of a molybdenum oxide which comprises incorporating a small proportion of ammonium molybdate with molybdenum oxide in powdered form in the presence of water, pressing the mixture, and drying the pressed product.

2. A process for the production of firm coherent masses of a molybdenum oxide which comprises adding to the molybdenum oxide in powder form a proportion of an aqueous solution of ammonia, pressing the mixture, and drying the pressed product.

3. A process as claimed in claim 1 in which the proportion of ammonium molybdate, calculated

as a percentage of  $\text{NH}_3$  by weight on the weight of the molybdenum oxide, lies between 0.05% and 2%.

4. A process as claimed in claim 1 in which the proportion of water lies between .7% and 5% by weight of the molybdenum oxide.

5. A process as claimed in claim 1 in which the pressing is conducted at a pressure lying between 2 and 20 tons per square inch.

10 6. A process as claimed in claim 1 in which the molybdenum oxide is molybdenum trioxide.

7. As a new article of manufacture, useful in the manufacture of alloys containing molybdenum, a firm coherent compacted mass of a composition consisting of molybdenum oxide containing a small proportion of ammonium molybdate intimately incorporated therewith as a binder.

15 8. As a new article of manufacture, useful in the manufacture of alloys containing molybdenum, a firm coherent compacted mass of a composition consisting of molybdenum oxide containing a small proportion of ammonium molybdate intimately incorporated therewith as a binder, said composition being substantially free from carbonaceous matter.

20 9. A process for the manufacture of alloys containing molybdenum which comprises adding to a molten metal bath containing a reducing agent in solution a firm coherent compacted mass of a composition consisting of molybdenum oxide containing a small proportion of ammonium molybdate intimately incorporated therewith as a binder.

25 10. A process as defined in claim 9, in which said composition is substantially free from carbonaceous matter.

GEORGE LESLIE MILLER.

40 REFERENCES CITED

The following references are of record in the file of this patent:

UNITED STATES PATENTS

| 45 | Number     | Name          | Date          |
|----|------------|---------------|---------------|
|    | Re. 12,643 | Ronay         | Apr. 30, 1907 |
|    | 900,587    | Ramsey et al. | Oct. 6, 1908  |
|    | 1,300,279  | Kissock       | Apr. 15, 1919 |
|    | 2,134,616  | Linz          | Oct. 25, 1938 |

50 FOREIGN PATENTS

| Number  | Country       | Date          |
|---------|---------------|---------------|
| 572,776 | Great Britain | Oct. 23, 1945 |